

1

2,902,416

## METHOD AND BATH FOR ELECTRODEPOSITION OF ALUMINUM

Arthur C. Doumas, Lake Jackson, Tex., and Nelson F. Murphy, Blacksburg, Va., assignors to Research Corporation, New York, N.Y., a corporation of New York

No Drawing. Application August 23, 1956  
Serial No. 605,713

9 Claims. (Cl. 204—14)

This invention relates to the electrodeposition of aluminum, and particularly to a process involving the deposition of aluminum on a suitable cathode and to a new and improved electrolytic bath therefor.

Aluminum electrodeposited on a base metal imparts the qualities of good appearance and high resistance to corrosion. Because of the excellent corrosion resistance of aluminum, protective coatings thereon on steel and other metals which are more easily corroded have been found to be highly desirable. In addition to the excellent corrosion resistance of aluminum, a process for aluminum plating could be used advantageously in easing the shortage of more critical plating materials, such as tin, of which there are no important deposits in the United States.

Processes for electrodeposition of aluminum on other metals have been developed in the past. However, many inherent unsolved problems have prevented their use in large-scale operation.

Various electrolytic systems for the deposition of aluminum have been carefully investigated which include organic solutions, aqueous inorganic solutions, non-aqueous inorganic solutions, and molten salt baths. It has been determined that it is not possible to electrodeposit aluminum from aqueous solutions because aluminum has a higher decomposition potential than hydrogen even at high hydrogen overvoltages. Molten salt baths have been employed in producing ductile, adherent deposits of aluminum when operated in a narrow range of compositions and conditions. However, molten baths containing aluminum chloride evolve copious fumes for which adequate means of disposal must be provided. Further disadvantages such as electrolyte degeneration, the high resistance of the bath and the low optimum current density result in slow and uneconomical deposits of aluminum.

In is a primary object of the present invention to provide a method of electrodeposition of aluminum and aluminum electrodeposition bath which is stable to moisture, inexpensive, and easy to control thereby providing a commercially feasible aluminum plating system.

A further object is to provide a process enabling aluminum to be electroplated on various base metals.

A further object of the present invention is to provide a novel electroplating bath which can be successfully and economically employed for electrodeposition of aluminum on a commercial scale. A still further object of the present invention is to provide a bath for the electrodeposition of aluminum which has a relatively high electrical conductivity, low voltage requirement and in which high electrode efficiencies are obtainable.

Yet another object is to provide an improved long life electrolyte for depositing aluminum on a metal or other electrically conductive surface.

In general, the bath for depositing the aluminum coating comprises an organic solution comprising alkylamines containing from one to three alkyl groups having a total of from four to twelve carbon atoms, an aliphatic ether,

2

including cycloaliphatic ether, containing from 4 to 6 carbon atoms, and aluminum chloride.

In general, the electroplating bath is prepared by dissolving a predetermined amount of aluminum chloride in one-half of the predetermined amount of aliphatic ether, and dissolving the predetermined amount of alkylamines in the other half of the aliphatic ether. The resulting solutions are cooled and then mixed. The mixture is then ready for use in a standard electroplating cell.

- 10 While it has been found that very satisfactory operation may be carried out in a closed cell at atmospheric pressures, it is not necessary to exclude air from the operation of this cell. However, if a closed cell is used and fitted with some form of cooled reflux condenser, 15 the loss of volatile components of the bath is prevented and the cell may be operated at higher temperatures. It is generally desirable to subject the cell to a period of electrolysis to eliminate impurities such as water and heavy metals at a current density of about 44 amperes per 20 square foot before electroplating of aluminum is commenced. The temperature of the electroplating bath may be varied over a wide range; for example, satisfactory results have been obtained with the temperature of the bath between ambient room temperature and the boiling 25 point of the particular solution. If higher temperatures are employed in the bath, it is necessary to provide means for condensing escaping vapors and returning the condensate to the bath as hereinbefore described.

- It will be seen from the specific examples presented 30 hereinafter that a wide range of mixtures of the alkylamines, aliphatic ethers and aluminum chloride provide satisfactory smooth, bright and adherent aluminum deposits. However, it has been found that most satisfactory results were obtained when the electroplating bath is 35 a single phase liquid mixture. For example, no deposits of aluminum are possible from mixtures which are solids at ordinary temperatures and the deposits of aluminum may be defective because of inclusions of solid particles, if the bath comprises a suspension of solids in liquids.
- 40 It has also been found that a wide range of current densities may be employed in the present electroplating process and the use of a periodically reversed direct current has in some instances provided brighter deposits than simple direct current.

- 45 When steel cathodes are employed in the process of the invention, smooth and bright finishes and a better adherence of the aluminum deposit is provided if the steel is provided with a preliminary deposit of zinc and this preliminary deposit of zinc may also be employed with 50 satisfactory results when plating aluminum on other metals than steel.

The following examples will serve to illustrate the invention with greater particularity.

Example I

55 A mixture comprising 28.0 mol percent aluminum chloride, 24.2 mol percent n-butyl amine, and 47.8 mol percent diethyl ether is prepared. The resulting oily liquid is placed in a suitable plating tank having an aluminum anode and a copper cathode. After a period of electrolysis for about 5 amp. hrs., to eliminate impurities at a current density of about 4.7 amperes per square decimeter, the bath was found to deposit a very satisfactory aluminum coat when the temperature of the bath was maintained at about 75° C.

Example II

An electrolytic solution is prepared consisting of 31.3 mol percent aluminum chloride, 31.3 mol percent n-butyl amine, and 37.4 mol percent diethyl ether. The solution was placed in a suitable plating tank and satis-

factory aluminum deposit on copper and steel was obtained when the bath was maintained at a temperature of from about 27° C. to about 75° C. employing an aluminum anode and cathode densities from about 1.13 to about 2.70 amperes per square decimeter.

*Example III*

Aluminum was electrodeposited on a steel cathode from an electrolytic bath consisting of 28.0 mol percent aluminum chloride, 24.2 mol percent n-butyl amine, and 47.8 mol percent diethyl ether, when the temperature of the bath ranged from about 27° C. to about 70° C., employing an aluminum anode and cathode current densities of from about 2.17 to about 2.69 amperes per square decimeter.

*Example IV*

Aluminum was deposited on a copper cathode from an electrolytic bath consisting of 14.0 mol percent aluminum chloride, 14.5 mol percent n-butyl amine, and 71.5 mol percent tetrahydrofuran when the bath was maintained at a temperature of from about 30° C. to about 75° C., employing an aluminum anode and a cathode current density of about 0.054 ampere per square decimeter.

*Example V*

Aluminum was satisfactorily electrodeposited on a copper cathode from an electrolytic bath consisting of 15.6 mol percent aluminum chloride, 13.6 mol percent 2-ethylhexyl amine, and 70.8 mol percent tetrahydrofuran when the bath was maintained at a temperature of from about 50° C. to about 95° C., employing an aluminum anode and a cathode current density of about 7.6 amperes per square decimeter.

*Example VI*

An electrolytic bath consisting of 21.5 mol percent aluminum chloride, 14.4 mol percent n-butyl amine, and 64.1 mol per cent n-propyl ether was found to provide satisfactory electrodepositions of aluminum on a copper cathode when the bath was maintained at a temperature of from about 25° C. to about 105° C., employing an aluminum anode and cathode current densities from about 0.78 to about 4.46 amperes per square decimeter.

*Example VII*

An electrolytic bath consisting of 16.0 mol percent aluminum chloride, 9.5 mol percent 2-ethylhexyl amine, and 74.5 mol percent n-propyl ether was found to provide satisfactory depositions of aluminum on a copper cathode when the bath was maintained at a temperature range of from about 95° C. to about 105° C., employing an aluminum anode and cathode current densities from about 0.60 to about 1.40 amperes per square decimeter.

*Example VIII*

An electrolytic bath consisting of 26.4 mol percent aluminum chloride, 18.2 mol percent n-butyl amine, and 55.4 mol percent n-butyethyl ether deposited satisfactory aluminum on a copper cathode when maintained in the temperature range of from about 60° C. to about 100° C., employing an aluminum anode and cathode current densities of from about 0.24 to about 13.74 amperes per square decimeter.

*Example IX*

Satisfactory deposits of aluminum on a copper cathode is provided from an electrolytic bath consisting of 25.9 mol percent aluminum chloride, 17.2 mol percent 2-ethylhexyl amine, and 56.9 mol percent n-butyethyl ether when the bath is maintained at a temperature of from about 85° C. to about 105° C., employing an aluminum anode and cathode current densities of from about 2.65 to about 4.70 amperes per square decimeter.

*Example X*

Aluminum was electrodeposited on a copper cathode from an electrolytic bath consisting of 40.0 mol percent aluminum chloride, 25.0 mol percent 2-ethylhexyl amine, and 35.0 mol percent diethyl ether when maintained at a temperature of from about 70° C. to about 110° C., employing an aluminum anode and cathode current densities in the range from about 1.85 to about 5.26 amperes per square decimeter.

*Example XI*

Aluminum was electrodeposited on a steel cathode from an electrolytic bath consisting of 40.0 mol percent aluminum chloride, 25.0 mol percent 2-ethylhexyl amine, and 35.0 mol percent diethyl ether when maintained at a temperature of from about 70° C. to about 110° C., employing an aluminum anode and cathode current densities in the range from about 1.85 to about 5.26 amperes per square decimeter.

*Example XII*

Aluminum was electrodeposited on a copper cathode with cathode current efficiencies of from about 7.5 to about 91.0 percent from an electrolytic bath consisting of 25.6 mol percent aluminum chloride, 15.2 mol percent 2-ethylhexyl amine, and 59.2 mol percent diethyl ether when the bath was maintained at a temperature of from about 85° C. to about 110° C., employing an aluminum anode and cathode current density in the range of from about 0.43 to about 7.78 amperes per square decimeter.

*Example XIII*

Aluminum was electrodeposited on a steel cathode with cathode current efficiencies of from about 7.5 to about 91.0 percent from an electrolytic bath consisting of 25.6 mol percent aluminum chloride, 15.2 mol percent 2-ethylhexyl amine, and 59.2 mol percent diethyl ether when the bath was maintained at a temperature of from about 85° C. to about 110° C., employing an aluminum anode and cathode current density in the range of from about 0.43 to about 7.78 amperes per square decimeter.

*Example XIV*

A deposit of aluminum on a zinc-plate copper cathode from an electrolytic solution consisting of 25.6 mol percent aluminum chloride, 15.2 mol percent 2-ethylhexyl amine, and 59.2 mol percent diethyl ether when the bath was maintained at a temperature from about 45° C. to about 60° C., employing an aluminum anode and cathode current densities of from about 1.28 to about 2.74 amperes per square decimeter.

*Example XV*

A deposit of aluminum on a zinc-plated steel cathode from an electrolytic solution consisting of 25.6 mol percent aluminum chloride, 15.2 mol percent 2-ethylhexyl amine, and 59.2 mol percent diethyl ether when the bath was maintained at a temperature of from about 45° C. to about 60° C., employing an aluminum anode, and cathode current densities of from about 1.28 to about 2.74 amperes per square decimeter.

From the foregoing description and the preceding examples, it will be seen that the process and electrolytic solution of the present invention provide means for obtaining electrodeposition of aluminum on base metals such as copper, iron, steel and the like and the invention is not to be limited to the particular illustrated embodiments hereinbefore set forth.

We claim:

1. An aluminum electroplating bath comprising a single phase liquid solution consisting essentially of from about 10 to about 45 mol percent aluminum chloride; from about 10 to about 40 mol percent alkylamine containing from one to three alkyl groups having a total of from

four to twelve carbon atoms, and from about 30 to about 80 mol percent of aliphatic ether containing from four to six carbon atoms.

2. The invention defined in claim 1 wherein the alkylamine comprises n-butyl amine and the aliphatic ether comprises diethyl ether.

3. The invention defined in claim 1 wherein the alkylamine comprises n-butyl amine and the aliphatic ether comprises tetrahydrofuran.

4. The invention defined in claim 1 wherein the alkylamine comprises ethylhexyl amine and the aliphatic ether comprises n-propyl ether.

5. The invention defined in claim 1 wherein the alkylamine comprises 2 ethylhexyl amine and the aliphatic ether comprises n-butyl-ethyl ether.

6. The invention defined in claim 1 wherein the alkylamine comprises 2 ethylhexyl amine and the aliphatic ether comprises diethyl ether.

7. The process of plating aluminum on dissimilar metals by electrodeposition which comprises subjecting, as 20 cathode, a metallic article to be plated, to the action of an electric current while immersed in a single phase liquid solution consisting essentially of from about 10 to about 40 mol percent alkylamine containing from 1 to 3 alkyl groups having a total of from 4 to 12 carbon atoms; from 25 about 30 to about 80 mol percent an aliphatic ether containing from 4 to 6 carbon atoms and from about 10 to about 45 mol percent of aluminum chloride.

8. An aluminum electroplating bath comprising a single phase liquid solution consisting essentially of from about 10 to about 45 mol percent aluminum chloride; from about 10 to about 40 mol percent of a primary alkylamine having a total of from 4 to 12 carbon atoms, and from about 30 to about 80 mol percent of an aliphatic ether containing from 4 to 6 carbon atoms.

9. The process of plating aluminum on dissimilar metals by electrodeposition which comprises subjecting, as cathode, a metallic article to be plated, to the action of an electric current while immersed in a single phase liquid solution consisting essentially of from about 10 to about 40 mol percent of a primary alkylamine having a total of from 4 to 12 carbon atoms; about 30 to about 15 80 mol percent of an aliphatic ether containing from 4 to 6 carbon atoms and from about 10 to about 45 mol percent of aluminum chloride.

#### References Cited in the file of this patent

#### UNITED STATES PATENTS

2,692,850 Safranek et al. \_\_\_\_\_ Oct. 26, 1954

#### OTHER REFERENCES

Journal of the Electrochemical Society, vol. 99, No. 6, pages 234-244.